

Jan. 16, 1951

C. L. MILTON, JR., ET AL

2,538,160

METHOD OF ELECTROFORMING MOLDS

Filed Aug. 1, 1949

4 Sheets-Sheet 1

Fig.1.



Fig.2.



RESINOUS POSITIVE OF HAND  
FILLED WITH MOLTEN WAX



Fig.7.



Fig.8.

Inventors

Clare L. Milton, Jr.  
Carl A. Nielson

George W. Gardner  
George H. Brown

334

ATTORNEYS

Jan. 16, 1951

C. L. MILTON, JR., ET AL

2,538,160

METHOD OF ELECTROFORMING MOLDS

Filed Aug. 1, 1949

4 Sheets-Sheet 2

Fig. 3.



Fig. 4.



Fig. 5.



Inventors

Clare L. Milton, Jr.  
Carl A. Nielson

George W. Gardner  
George W. Gardner

ATTORNEYS

354

Jan. 16, 1951

C. L. MILTON, JR., ET AL  
METHOD OF ELECTROFORMING MOLDS

**2,538,160**

Filed Aug. 1, 1949

4 Sheets-Sheet 3



## Inventors

Clare L. Milton, Jr  
Carl A. Nelson

Carl A. Nielson  
George W. Gardes  
Joseph H. Brown

**ATTORNEYS**

Jan. 16, 1951

C. L. MILTON, JR., ET AL

2,538,160

METHOD OF ELECTROFORMING MOLDS

Filed Aug. 1, 1949

4 Sheets-Sheet 4

Fig. 10.



Fig. 11.



Fig. 12.



Inventors

Clare L. Milton, Jr.  
Carl A. Nelson

George W. Gardes  
Joseph M. Brown  
834

ATTORNEYS

## UNITED STATES PATENT OFFICE

2,538,160

## METHOD OF ELECTROFORMING MOLDS

Clare L. Milton, Jr., Roslyn Heights, N. Y., and  
Carl A. Nielson, Takoma Park, Md., assignors  
to the United States of America as represented  
by the Secretary of the Army

Application August 1, 1949, Serial No. 107,978

4 Claims. (Cl. 204—6)

(Granted under the act of March 3, 1883, as  
amended April 30, 1928; 370 O. G. 757)

1

The invention described herein may be manufactured and used by or for the Government for governmental purposes, without payment to us of any royalty thereon.

The present invention relates to a process of producing metal molds for use in casting plastic resinous objects by electrodeposition of the metal on a flexible model.

The molds of the present invention are adapted more specifically to the casting of objects of highly complex shapes, which duplicate, in high fidelity, an original model object. When the object to be reproduced is so detailed that machining is impossible or uneconomical, recourse is taken to producing a mold by spraying, casting, or electroforming. If, in addition, a moderately strong or dense deposit of a high-melting metal is required, and the object to be reproduced is of such a shape that not all of the areas can be sprayed at an angle of approximately 45°, satisfactory molds can be produced only by casting, or by electroforming.

The present invention relates to a method of electroforming a mold which is particularly advantageous in the casting of a natural-appearing glove for covering a prosthetic hand, or in any application wherever major undercuts are encountered.

The process of the present invention comprises conducting the electroforming over a hollow, flexible model of the object to be reproduced by the mold, the interior cavity of the mold duplicating in high fidelity the surface details of the object to be duplicated, the said model being filled with a readily removable, rigidifying core capable of being dissolved, softened, or melted, to the extent that it may be removed at a temperature below the temperature of decomposition or melting of the hollow flexible model, or the temperature at which appreciable distortion of the electroformed mold would take place.

For example, there is shown in the accompanying drawings a series of steps employed in the making of a mold for the production of such seamless gloves, in which the characteristics of size, contour and surface details of a natural hand are reproduced in high fidelity; and while the invention is not limited necessarily to such embodiment, the invention was developed with such embodiment as its primary aim and purpose.

It is apparent that when an individual has lost one or both hands and is fitted with an artificial hand as a prosthetic device for replacement of the missing member, there is afforded an im-

2

portant uplift in morale if the prosthetic appliance can be rendered inconspicuous to an observer. The usual kid gloves employed as the conventional coverings for such artificial hands only serve to advertise to the public the deformity of the wearer. The process of the present invention provides, among other things, the production of a glove for such purpose that renders the artificial hand indistinguishable to an observer

10 from a natural hand.

In order to accomplish such a desirable result, certain procedures must be followed, and as applied to the production of a glove which is virtually indistinguishable from a natural hand, the process of the invention comprises the following general steps:

1. The formation of an initial impression of a selected "model" hand of an individual whose natural hands match in size and shape, as closely as possible, the natural hand of the amputee. Thus, if the amputee is a unilateral amputee, that is, one who has lost only one hand, the remaining hand is matched as closely as possible as to size and shape by the hand of an individual who is selected to serve as a model. Thus, if the right hand of the amputee is missing, there is selected as a model an individual whose natural right hand matches the size and contour of the amputee's left hand as closely as possible. If the amputee is bilateral, i. e., has lost both hands, such a close matching of size and contour is not so important and the initial impression is made of both hands of the individual chosen as the model.

2. The initial impression of the model's hand duplicates the shape and surface characteristics of that hand. When the impression has been formed, the hand is removed, and the resulting cavity is filled with a selected resinous composition which is liquid when introduced into the impression, but which can be coagulated or gelled readily on the surfaces of the impression. The ungelled, liquid residual resin is removed from the impression leaving the resulting gelled resinous "skin" in place in the cavity of the original impression. This resinous skin is a positive of the impression and it is reinforced preferably before it is removed from the impression, by filling it with a rigidifying core, such as molten wax, which is allowed to solidify in the gelled resin positive. A suitable electrode hanger is inserted in the rigidified core, and the whole assembly is removed from the original impression. The positive gelled resinous "skin" is made electrically conductive and is placed as cathode in an electro-forming bath, preferably an aqueous bath of

nickel or copper salts, and electropated with metal under controlled conditions which assure a uniform deposit of metal all over the conductive positive "skin." When a suitable thickness of metal is deposited, the plated assembly is removed from the bath, the wax is removed by melting and draining it out through the wrist opening, the positive skin then is separated mechanically from the interior of the metal deposit, and pulled out through the said wrist opening, leaving the deposited metal as a seamless mold which duplicates interiorly the surface characteristics of the original model hand, and in which the final composition is adapted to be cast.

Reference now may be had to the accompanying drawings in which:

Fig. 1 is a diagrammatic view illustrating a model hand inserted in a bath adapted to form the initial impression which is employed in producing the mold in accordance with this invention;

Fig. 2 is a diagrammatic view showing the initial impression of the model hand, with the hand removed;

Fig. 3 is a diagrammatic view of the original impression filled with liquid resin for forming the positive;

Fig. 4 is a view similar to Fig. 3, but showing peripheral gelation of the resin in the impression;

Fig. 5 is a view similar to Fig. 4, but showing ungelled resin being removed from the initial impression;

Fig. 6 is a view similar to Fig. 5, but showing the resin completely removed from the gelled positive, which is still in the original impression;

Fig. 7 is a view similar to Fig. 6, but showing the gelled positive filled with a rigidifying core, such as molten wax;

Fig. 8 is a view showing the positive and solidified wax core removed from the initial impression bath, with a fragment of an electrode hanger inserted therein, the resulting form being provided with an electroconductive coating;

Fig. 9 is a diagrammatic perspective view of a preferred form of plating equipment for electro-forming the mold of the present invention, the view showing the electrical connections of the deposition cell;

Fig. 10 is a longitudinal, vertical, sectional elevation of the cell of Fig. 9, the view being taken on the vertical longitudinal center line of the cell of Fig. 9;

Fig. 11 is a transverse sectional plan view through the wrist portion of the form being plated in Fig. 9, the view indicating the layer of deposited metal, the rigid core material for the form being still in place;

Fig. 12 is a view similar to Fig. 11, but with the rigid core material removed, and showing the resinous positive prepared as outlined above, separated from the deposited metal and collapsed for removal from the resulting electrode-deposited mold; and

Fig. 13 is a fragmentary sectional elevation of an auxiliary anode illustrated in Fig. 10, showing details of protective insulation on the anode, with electrical connection to the anode, the view being applicable to either auxiliary anode shown in Figs. 9 and 10.

Referring more particularly to the drawings, the numeral 12 represents a model hand immersed in a bath 14 for forming an initial impression of the hand. The bath 14 is contained in a suitable receptacle 15, and is a gelable liquid alginate composition that is adapted to gel about

the hand to form a stiff, elastic gelled mass, the hand forming an impression therein which duplicates in the surfaces of the impression all surface details of the model hand. Since it is a requisite that the model hand 12 be releasable from the elastomer gelled alginate bath 14 without permanent distortion of the impression of the hand, the composition of this material is critical, not only because of the requisite elastic properties of the gelled material, but because of the fact that gelation of the material must be effected at a temperature sufficiently low to prevent discomfort to the individual whose hand is serving as the model. When gelled, however, the bath must resist liquefaction at temperatures above the gelation temperature of the positive-forming resin which is to be introduced into the impression.

In practice, the bath 14 is made satisfactorily of a liquid alginate which can be obtained from kelp. It is found in practice that the material sold on the market as "Coe-loid" duplicating colloid material is well suitable, this colloid being a polymer of d-manuronic acid extracted from kelp. This alginate material is incorporated in an aqueous retarder solution and water, the retarder solution retarding the gelation of the alginate until the model hand 12 is introduced into the bath and properly positioned. The retarder solution is composed of a mixture of sodium phosphates, calcium phosphates and potassium phosphates, the concentration of the phosphates depending upon the desired length of gelation time. Thus, for example, a bath made up in the proportions of 13.5 gms. of "Coe-loid" duplicating colloid (alginate), 70 cc. of retarder solution containing about equal amounts by weight of sodium, calcium and potassium phosphates to substantial saturation, and 30 cc. of water will form a stiff elastomeric gel in about ten minutes at a temperature of from 35° to 40° C. The time of gelation can be controlled by the amount and concentration of the retarder solution employed, the more retarder the slower the time of gelation. The d-manuronic acid may be regarded as being synonymous with alginic acid. The resulting material is sufficiently elastic when gelled to permit the model hand being withdrawn from the gelled bath without permanent distortion of the impression or injury to the detail lines corresponding to the surface features of the model hand. Upon removal of the hand, the material which is stretched during such removal returns to its original position, leaving the impression cavity 16 as a duplicating negative impression of the hand 12. Since the hand 12 is immersed in the bath above the wrist portion 18, when the hand is withdrawn, the opening 22 in the cavity 16 returns to the size of the arm portion which was immersed in the bath while liquid. The impression 16 is a high-fidelity duplicate of the hand 12 down to minutest details of surface characteristics, including veins, knuckles, nails and finger print lines, the impression being, however, reversed (negative) with respect to the hand 12. Withdrawal of the model hand 12 is effected by gently working the fingers and hands loose from the encasing gel, cold water being poured around the hand during this operation, if desired, to further rigidify the gel and contract it away from the fingers and hand. Also, compressed air may be introduced into the cavity 16 as the hand is withdrawn in order to neutralize any tendency to form a vacuum in the cavity behind the fingers and hand as the hand is withdrawn.

The impression 16 forms a mold for casting a flexible resinous positive which forms the foundation for the finished mold produced in accordance with this invention. For forming this flexible positive, the impression cavity 16 is filled with a resinous composition 22 which gels under moderate heat supplied from a source of heat 24. The resinous composition 22 preferably is a dispersion of polyvinyl chloride or a copolymer of vinyl chloride with vinyl acetate, methyl or ethyl acrylate, methacrylate, fumarate or maleate, vinylidene chloride or other monomers, the polymer or copolymer, containing at least thirty-five percent of chlorine, in a solution containing from 0.5 per cent to five per cent of a polymer or copolymer selected from the group above, or a polymer of one of the monomers mentioned above, the balance of the solution being made up of a plasticizer for the chlorine-containing resin. There may be used also compositions similar to the above in which the chlorine-containing resin is dispersed in a plasticizer or mixture of plasticizers alone, rather than in a solution of a polymer in such a plasticizer.

The following examples indicate examples of resinous compositions suitable for the production of the above-indicated flexible positive, the proportions being parts by weight:

*Example I*

|                                                        | Parts |
|--------------------------------------------------------|-------|
| Paste grade polyvinyl chloride-vinyl acetate copolymer | 100   |
| Tricresyl phosphate                                    | 25    |
| Dibutyl phthalate                                      | 25    |
| Polyethyl methacrylate                                 | 4     |

*Example II*

|                                                        | Parts |
|--------------------------------------------------------|-------|
| Paste grade polyvinyl chloride-vinyl acetate copolymer | 40    |
| Di-2-ethylhexyl phthalate                              | 29    |
| Tricresyl phosphate                                    | 29    |
| Polyethyl methacrylate                                 | 2     |

*Example III*

|                                            | Parts |
|--------------------------------------------|-------|
| Polyvinyl chloride resin                   | 45    |
| Di-2-ethylhexyl phthalate                  | 26.7  |
| Tricresyl phosphate                        | 26.7  |
| Polyvinyl chloride-vinyl acetate copolymer | 1.5   |

The foregoing compositions are free-flowing and gel at moderate temperatures, for example, from about 60° C. to about 90° C. The alginate bath 14 has the characteristic of being permanent at such gelation temperature of the resin. This alginate bath may be warmed to its gelation temperature of 35° to 40° C., by a source of heat 24, if need be, for forming the initial impression.

Upon heating the bath to gelation temperature of the resin 22, the resin composition gels peripherally as indicated at 26, this forming a gelled resinous "skin" which is a positive duplicate of the original impression 16. The ungelled resin 22 is removed, as by decantation or syphoning through a tube 28, and the gelled skin, which is left undisturbed in the impression is built up to a requisite thickness by refilling with the resinous dispersion, gelling additional resin on the skin and removing ungelled resin as before, this procedure being repeated as many times as may be necessary to build up the desired thickness of deposit. This repeated procedure is preferred to avoid the possibility of over-heating the gelled portion of the resin or the alginate bath.

Upon completion of the gelation, there remains in the impression 16 a fragile, gelled positive

replica of the impression and therefore of the original hand. This positive replica 26, being of a fragile character, is reinforced, preferably before it is removed from the impression, by filling it with molten wax as is indicated at 30, which wax has a low melting point, and which is allowed to solidify in the positive skin 26, thereby rendering this positive replica rigid for the insertion of an electrode hanger 32, and also to enable the positive replica to be handled more readily without tearing. The rigidifying matrix 30 is selected from such compositions as will be removable readily from the final mold. Preferably the wax is chosen so that it will melt below the boiling point of water. However, a mixture of such wax with sand, or a wax-clay mixture, or an oil-clay mixture may be used as the rigidifying matrix. However, a sand-wax mixture is preferred because it possesses the advantages that it does not shrink appreciably on cooling, that it retains the shape when the filled resinous model is immersed in hot water, and when warm it is sufficiently soft to permit any desired repositioning of the model. Thus, when the flexible hollow model 26 of the hand is filled with a mixture of sand and wax, removed from the alginate bath and warmed, the fingers may be adjusted into whatever position is regarded as most desirable, and on cooling, this position is retained in the now-rigid model; yet in spite of this highly desirable plastic property, the mixture of sand and wax can be washed out readily with hot water. It is desirable for successful electroforming, that the form be sensibly rigid during the period of plating.

When the rigidifying core 30 has hardened, the resulting form is removed from the alginate bath 14. This is the preferred procedure, although the invention contemplates a removal of the positive 26 from the gelled alginate bath 14 prior to filling the positive form with the rigidifying material. When the rigidifying material has hardened, either with the positive 26 still in the impression 16 or removed therefrom, the hanger 32 is inserted. It will be understood that when the resinous positive 26 has been formed in the impression 16, the alginate bath 14 has served its purpose, and the destruction of the impression incident to removal of the positive 26 is immaterial.

In order to deposit the mold-forming metal onto the resinous positive form 26, the surfaces thereof must be rendered electrically conductive. For this purpose, an electrically conductive coating 34 is applied to the surfaces of the positive form 26. Thus, for example, the coating may be a very thin layer of metallic silver applied by spraying the positive form with ammoniacal silver nitrate, thereby producing a continuous coating of metallic silver on the form which is at most only a few molecules in thickness for avoiding masking any of the fine surface lines on the positive 26.

The coating 34 is a continuous coating and is sufficiently adherent to the resinous positive to stay in place when the positive form is introduced into the electroforming bath. The final mold metal may be any metal of high melting point that may be deposited from an aqueous bath, and which metal is inert to polyvinyl chloride. Thus the preferred metal is nickel, backed, if desired, with either copper or iron.

The production of the final mold by electroforming operations is shown by Figs. 9 through 13 of the accompanying drawings.

In these views, the form, indicated at 40, with

its surface rendered electrically conductive, is suspended as a cathode by hanger 32 in an electrolytic cell containing as electrolyte, an aqueous solution of the metal to be deposited. When nickel is such metal, the well-known Watts bath may be employed as electrolyte, although an all chloride type of nickel bath may be employed with excellent results, and the various addition agents used in bright nickel electroplating are beneficial in this application. Suspension of the form 40 is effected by the hanger bar 32 thrust into the wax core 30, the bar 32 being clamped to the cathode bus bar 42 by a clamp 43 for intimate contact with the bus bar, the conducting surface of the form 40 being connected to the hanger bar 32 by a coil of wire 44 wrapped around the form and connected by a conducting lead 46 to the cathode hanger bar 32, as indicated by contact screw 48.

Current is supplied from plating anodes 50, 52, suspended from the anode bus bars 54, 55, these anodes being plates of the metal being deposited, the anode plates 50, 52 preferably being positioned on both sides of the form to facilitate the production of uniform deposit of the metal on the surface of the form 40. The anodes 50, 52 are suspended from the bus bars 54, 55 by hooks 56, 58, which intimately engage the bus bars 54, 55 in the well-known manner.

Also, in order to prevent excessive thickness of metal being deposited on the ends of the form, an auxiliary cathode or "thief" 60 may be provided, connected by leads 62 to the cathode hanger bar 32 for "stealing" metal from the ends of the fingers of the form, there being thus obtained a uniform deposit of metal over the positive 26. The auxiliary cathode or "thief" may be simply a single wire spaced from the finger tips of the form and roughly conforming to the contour of the form. The auxiliary cathode wire 60 may be provided with a protective lacquer layer 61 except for the exposed length of the wire which encloses the form. Auxiliary anodes also may be provided; for example, there may be an anode 63 between each finger of the form connected by the leads 65 to the anode lead 66, thence to the anode side of the power line through lead 67 to ammeter 68 and rheostat 70, as shown. The plating anodes 50, 52 are connected to the anode side of the power line through ammeter 72 and rheostat 74. It will be seen also that an auxiliary anode 76 is directed towards the palm of the form and spaced therefrom a suitable distance for assuring uniform deposition of the metal on the palm of the form. This anode is connected to the anode side of the power line through lead 78, ammeter 80, and rheostat 82. Except for the desired areas for plating, the auxiliary anodes are provided with an insulating sheath, such as rubber, 84, which is lacquered as indicated at 86, the insulating coating being interrupted at 88 for attachment of the leads 67 and 78.

After completion of the electrodeposition, the form consisting of the rigidifying core 30, intermediate resin positive 26, conductive coating 34 and deposited metal 90, is removed from the plating bath. The rigidifying core 30 is removed by melting the wax and sluicing out with hot water, the resinous positive 26 then being collapsed as indicated in Fig. 12, and pulled out from the deposited metal through the open wrist portion thereof, the inner surfaces of the resulting metal mold accurately duplicating all details of the resinous positive.

The metal deposit 90 may be nickel only, or a multiple coating of different metals, such as nickel backed by copper. Thus, where the hollow metal form is to be employed as a mold for casting plastic "cosmetic" gloves, the single layer of nickel may be 0.020 inch thick, or if made of multiple coatings, a layer of nickel 0.005 inch thick may be deposited first, covering this with 0.020 inch of copper and overlaying this copper with 0.002 inch of nickel.

After removal of the rigidifying core and the flexible positive, the mold may be cleaned by dipping into nitric acid followed by washing with ammonia and water.

15 The arrangement of the plating cell as shown in the accompanying drawings permits a close control of the plating current to be supplied to the anodes, and the illustrated disposition of the electrodes assures a uniform deposit of metal over the form, which is desirable for obtaining uniform heat conductivity through the mold, as where the finished mold is to be used in the forming of gloves to be used as natural-appearing coverings for mechanical hands, the cast resin is to be heated in the mold at elevated temperatures for sufficient time to cure and vulcanize the cast shape.

While the specific embodiment of the invention herein illustrated and described is applied to the production of molds shaped like a human hand for the production of gloves duplicating a natural hand in texture, appearance, and surface characteristics, as has been described above, the process actually is of general application. In the production of a glove for covering a mechanical hand, it is a requisite for natural appearance, to duplicate in the finished glove all surface details of a natural hand, such as palm and finger lines, finger nails, veins and the like, which can be obtained by making the negative impression of a model human hand in the gelable liquid material and causing the liquid to gel on and around the hand while it is immersed in the solution. The resulting gelled material is sufficiently elastic to permit the hand to be withdrawn by gentle muscular movement without permanent distortion or defacement of the impressed surface characteristics of the hand, the gelable liquid being of sufficiently low viscosity to fill all surface characteristics and irregularities of the model natural hand. The liquid bath gels on standing a predetermined short time, of the order of ten minutes or less, at approximately 35° C. to 40° C., there remaining when the hand is withdrawn, a high-fidelity duplicate of the hand, as a hollow impression in the gelled bath, this impression being a negative of the hand, and being open corresponding to the wrist or arm portion of the hand, the impression duplicating the hand and as much of the wrist and arm as may have been immersed in the liquid. Accordingly, the impression and the resin positive model will be hollow and co-extensive with the depth of immersion of the hand and arm. It is this resinous positive which is rigidified by introducing the wax-sand mixture or wax before the resin positive is removed from the gelled negative impression, and since the rigidified positive is sufficiently tough to permit its being handled, it, together with its filling, can be removed and is electroplated as described herein to form the mold. As the metal is electrodeposited from an aqueous electrolyte, and since the deposit forms initially as a continuous monomolecular deposit, the finished metal mold, after the rigidifying core has been melted and drained

through the open wrist portion of the form, and the resinous positive collapsed and removed through this same opening, duplicates interiorly all of the surface details of the original negative impression, and therefore of the model natural hand.

It will be understood that the form being plated may not be the shape of a human hand, but can be of any other shape; and the particular configuration of the object being plated is determinative of the number, arrangement, and composition of the electrodes, and also the composition of the plating bath. It is necessary, however, that the model being plated is flexible, hollow, and open, so that the rigidifying core can be removed through the opening, and the model collapsed away from the electrodeposited coating and pulled out through that opening. It will be understood that the portion of the rigidifying core which fills the opening in the flexible model will not be plated, so that the continuity of the plating will be interrupted to this extent, and there is left an opening through which the core material when liquefied can be drained; and such opening permits access to the flexible resinous positive for separation thereof from the deposited metal and withdrawal thereof from the hollow interior of the deposited metal which is left as a hollow, seamless, one-piece metal mold interiorly duplicating in high fidelity all of the surface details of the flexible positive.

The metal of the mold is dependent on the composition of the final cast product, as has been mentioned above. Thus, if the final composition is not a chlorine-containing resin, the mold may be composed of electrodeposited copper. Choice of metal is determined by inertness to the final composition to be cast in the mold, the refractoriness of the metal to heat (resistance to melting and oxidation) and ease of deposition from aqueous electrolytes.

Where a glove duplicating a natural hand is being made, the wax core of the form is exposed at the wrist or arm opening in the resin positive, and this exposed end of the rigidifying core is not conductively coated, so that the electrodeposited metal is interrupted to form an opening in the deposited mold corresponding to this exposed wax, the resulting opening permitting drainage of the molten core, and removal of the resin positive. In the case of other forms, the electrodeposited metal is interrupted by stopping off or masking a portion of the form being coated to make the electrodeposited metal discontinuous over such predetermined areas for providing an opening for the removal of the core and positive.

The process of this invention includes the foregoing manipulative steps generally, as well as the steps and critical factors involved in the application of the process to the production of prosthetic gloves duplicating in high fidelity detail the texture and appearance of a natural hand. It will be apparent, therefore, that it is intended and desired to embrace within the scope of this invention such modifications and changes as may be necessary to adapt it to varying conditions and uses, as defined in the appended claims.

The present application is a continuation-in-part of copending application Serial No. 5,712, filed February 2, 1948, for Process for Making Molds, now abandoned.

Having thus described our invention, what we claim as new and wish to secure by Letters Patent is:

1. In the production of seamless cosmetic gloves

for covering prosthetic hands, the steps which comprise immersing a model natural hand in a congealable liquid alginate composition which forms a stiff, elastic gel when congealed, congealing the composition around the hand and adjacent arm portions, thereby producing an impression in the congealed alginate gel which duplicates all surface characteristics of the model hand, removing the hand from the impression without permanently distorting the impression and lines therein duplicating the surface characteristics of the model hand, producing an open, flexible positive of the model hand from the said impression by filling the impression with a congealable liquid resinous composition including a polymerized vinyl resin dispersed in a plasticizer therefor, and which gels at a temperature below the liquefying temperature of the alginate to form a flexible, elastic gel, congealing the resin on the periphery of the impression, removing residual ungelled resin from the impression while leaving the resulting flexible positive in the said impression, filling the resulting open, seamless, flexible positive with a readily removable rigidifying core, removing the resulting rigidified positive from the said impression, rendering the positive electrically conductive, electrodepositing a mold metal on the rigid positive except over portions of the core exposed by the opening in the positive, thereby producing an open, electrodeposited mold form through the opening in which the core and flexible positive can be removed, and removing the core and flexible positive from the electrodeposited metal through the said opening, thereby leaving a hollow seamless, open metallic mold interiorly duplicating the surface characteristics of the original model hand.

2. In the production of seamless cosmetic gloves for covering prosthetic hands, the steps which comprise immersing a model natural hand in a congealable liquid alginate composition which forms a stiff, elastic gel when congealed, congealing the composition around the hand and adjacent arm portions, thereby producing an impression in the congealed alginate gel which duplicates all surface characteristics of the model hand, removing the hand from the impression without permanently distorting the impression and lines therein duplicating the surface characteristics of the model hand, producing an open, flexible positive replica of the model hand from the said impression by filling the impression with a congealable liquid resinous composition including a polymerized vinyl resin dispersed in a plasticizer therefor, and which gels at a temperature below the liquefying temperature of the alginate to form a flexible, elastic gel, congealing the resin on the surfaces of the impression, removing residual ungelled resin from the impression while leaving the resulting flexible positive in the said impression, filling the resulting open, seamless, flexible positive with a molten wax composition having a low melting point, hardening the wax composition in the positive to rigidify the positive, removing the resulting rigidified positive from the said impression, rendering the rigid positive electrically conductive, suspending the rigid positive as cathode in an electroforming bath, electrodepositing metal from the bath onto the positive except on the exposed portion of the core until the positive is coated uniformly with the metal, thereby producing an open coating of metal on the positive, removing the coated positive from the bath, melting and draining the wax rigidifying composition from the coated positive through

the opening in the coating, collapsing the flexible positive away from the coating metal, and withdrawing the collapsed positive through the said opening thereby leaving a hollow metal mold replica of the positive adapted to receive a resinous glove composition for molding therein cosmetic gloves to cover prosthetic hands.

3. The process of producing hollow, seamless molds for reproducing objects of intricate shapes, which comprises immersing the initial object to be introduced into a liquid alginate bath composition which forms a stiff elastic gel when congealed, effecting gelation of the composition about the object, removing the object from the gelled alginate bath, thereby leaving an initial impression of the object in the gelled alginate bath, introducing into the impression a fluid gelable resinous composition comprising essentially a polymerized vinyl resin dispersed in a plasticizer therefor and having a gelation temperature below the melting point of the gelled bath, effecting gelation of the resin over the peripheries of the impression, withdrawing ungelled residual resin from the said impression, thereby producing a flexible open positive of the impression, filling the positive with a rigidifying core including a low melting point wax, removing the rigidified positive from the alginate impression, coating the positive exteriorly with an electrically conductive material while the core is still in the positive, suspending the resulting coated and rigid positive as a cathode in an electro-forming bath, depositing metal on the positive until the positive is coated with the electrodeposited metal while controlling deposition of the metal to produce a uniformly thick coating of metal on the positive over all coated surfaces thereof, removing the electrodeposited form from the electroforming bath, melting out the rigidifying core through an opening in the coating corresponding to an uncoated portion of the positive, collapsing the flexible positive away from the deposited metal, and removing the resulting collapsed positive through the said opening, thereby leaving the deposited metal as a rigid, hollow metal mold interiorly duplicating all details of the initial impression.

4. The process of making hollow, seamless, metal molds for duplicating objects of intricate shape, which comprises immersing an object to be duplicated in a gelable but fluid bath of an alginate composition, effecting gelation of the bath around and on the object to be duplicated, removing the object from the resulting gelled

bath thereby leaving an open, gelled initial impression of the object, introducing into the impression a gelable resinous composition comprising a flowable mixture of polymerized vinyl resin and a plasticizer therefor and having a gelation temperature below the melting point of the gelled alginate bath, to yield upon gelation a flexible elastic resin gel, heating the resinous composition in the impression until peripheral gelation of the resinous composition is effected on the surfaces of the impression, removing ungelled resinous composition from the impression, thereby leaving an open resinous positive of the object of the impression, rendering the resulting flexible positive rigid by introducing therein a liquid low melting point core material and solidifying the core material in the positive, removing the positive from the impression, applying a coating of electrically conducting material to the exterior surface of the positive, introducing the rigidified positive as a cathode in an electroforming bath, electrodepositing metal on the coated surfaces of the positive, thereby producing a seamless, open electrodeposit on the positive, removing the resulting electrolytically coated positive from the electroforming bath, melting the core, draining the resulting molten core material from the electroformed metallic coating, collapsing the flexible resinous positive from the said metallic coating, and removing the collapsed resinous positive from the interior of the said coating through the opening therein, thereby leaving the coating as a rigid, hollow, seamless, metal mold interiorly duplicating all surface details of the initial impression of the object being reproduced.

CLARE L. MILTON, JR.  
CARL A. NIELSON.

## REFERENCES CITED

40 The following references are of record in the file of this patent:

## UNITED STATES PATENTS

| Number    | Name  | Date          |
|-----------|-------|---------------|
| 1,296,498 | Fodor | Mar. 4, 1919  |
| 2,124,871 | Beal  | July 26, 1938 |
| 2,275,582 | Bull  | Mar. 10, 1942 |

## OTHER REFERENCES

50 Molding and Casting, by Carl Dome Clarke, 2nd ed., 1946, pp. 135-138, 291-294.  
Acrylics, by S. D. Tylman and F. A. Peyton, 1946, pp. 141-144.